

July 3, 1951

N. W. KNEWSTUBB ET AL  
ROD COMPRISING BONDED FIBROUS MATERIAL  
AND METHOD OF MAKING SAME

2,558,855

Filed March 3, 1945

2 Sheets-Sheet 1

*Fig. 1.*



*Fig. 2.*



*Fig. 3.*



*Fig. 4.*



*Fig. 5.*



*Fig. 6.*



*Fig. 7.*

INVENTORS  
NORMAN WATSON KNEWSTUBB  
CHARLES ALEXANDER ROBB

BY *Escheller*  
ATTORNEY

July 3, 1951

N. W. KNEWSTUBB ET AL  
ROD COMPRISING BONDED FIBROUS MATERIAL  
AND METHOD OF MAKING SAME

2,558,855

Filed March 3, 1945

2 Sheets-Sheet 2

Fig. 9.



Fig. 10.

Fig. 11.



INVENTORS  
NORMAN WATSON KNEWSTUBB  
CHARLES ALEXANDER ROBB

BY *O. Scheffler*  
ATTORNEY

## UNITED STATES PATENT OFFICE

2,558,855

## ROD COMPRISING BONDED FIBROUS MATERIAL AND METHOD OF MAKING SAME

Norman Watson Knewstubb, Solihull, Birmingham, and Charles Alexander Robb, Moseley, Birmingham, England, assignors, by mesne assignments, to Union Carbide and Carbon Corporation, a corporation of New York

Application March 3, 1945, Serial No. 580,912  
In Great Britain March 6, 1944

13 Claims. (Cl. 154—91)

1

This invention is for improvements in or relating to rods comprising bonded fibrous material.

A rod of this type is normally prepared by rolling a sheet of fibrous material such as paper or textile material, which has been treated with binder, around a mandrel of small cross-sectional area, extracting the mandrel and then subjecting the resulting tube-like element to combined heat and mechanical pressure in such a manner that the tube collapses and a solid rod results. A disadvantage associated with this method is that the collapsing of the tube-like element is seldom completely effected and thus the material at the core of the rod tends to be of lower density than the rest of the rod and another disadvantage is that normally the application of sufficient pressure to collapse the tube requires the use of rigid and expensive dies which are necessarily limited in regard to length.

It is an object of the present invention to provide a simple and efficient method of preparing rods free from the disadvantages above referred to.

According to the present invention, a process for the manufacture of rods comprising bonded fibrous material includes the steps of impregnating and/or coating longitudinally-arranged fibres or fibrous elements with a bonding agent and applying twist and tension to a bundle of the treated fibres and, if necessary, heating to effect bonding of the fibres.

The term "longitudinally-arranged fibres or fibrous elements" is used in this specification to include filaments, slivers, rovings, yarns, threads, cables, strings and ropes, and also string-like elements prepared by twisting, felting or woven fibrous materials. The fibres may be organic or inorganic, natural or synthetic. For convenience of handling, the fibres may be enclosed within a sheath or tube of woven material.

Fibrous material in sheet or tape form and treated with bonding agent may be wound around the twisted longitudinally-arranged fibres or fibrous elements before, during, or after the latter have been subjected to heating, so that in the resultant rod the longitudinally-arranged fibres form a solid core.

After the longitudinally-arranged fibres or fibrous elements have been impregnated with a bonding agent, the content of the latter may be controlled by passing the impregnated fibres through a die or through squeeze rolls to eliminate surplus binder.

Twist and tension may be applied to the fibres or fibrous elements simultaneously.

2

The rods of the present invention, unlike those made by conventional methods, are not limited in length by the dimensions of available moulds, but may be prepared in continuous lengths.

- 5 The bonding agent may be organic or inorganic such as sodium silicate or Portland cement. It may consist of resinous material which may be thermoplastic (such as colophony, shellac, cellulose derivatives or polymerisation products) or 10 may be thermosetting (such as the condensation products of formaldehyde with a phenol, a urea, or an aminotriazine). The bonding agent may be a rubber-like material and may include natural or synthetic rubber.
- 15 Following is a description by way of example only and with reference to the accompanying diagrammatic drawing of methods of carrying the invention into effect.
- In the drawing:
- 20 Figure 1 shows a hank of cotton yarn 11 supported by a cord 12 and undergoing impregnation with an aqueous solution of a heat-hardenable phenol-formaldehyde condensation product in a bath 13.
- 25 Figure 2 shows the hank 11, after removal from bath 13, being passed through a die 14 for the removal of surplus liquid.
- Figure 3 shows, as an alternative to the die of Figure 2, adjustable squeeze rolls 15, 16 for the removal of surplus liquid from the impregnated hank.
- 30 Figure 4 shows the impregnated hank 11 suspended in a drying oven fitted with heating means 18 and a thermometer 19.
- 35 Figure 5 shows the dried impregnated hank suspended from a hook 20 in an oven 21 and subjected to tension by means of a weight 22 fitted with a bar 23 for subsequent rotation of the weight. The oven is provided with heating means 24, thermometer 25 and sockets 26 and 27 to receive posts for locking the bar 23 against rotation.

- 40 Figure 6 is similar to Figure 5 except that twist in the impregnated hank 11 has been imparted by twisting the weight 22 by means of the bar 23 and the bar has been locked against untwisting by the insertion of posts 28, 29 in the sockets 26 and 27.

- 45 Figure 7 shows excess of hardened resin on the surface of the cured and twisted hank 11 being removed by a machining operation to produce a finished rod as at 30.

- 50 Figure 8 shows a finished rod as 30 (Figure 7) which has been used as a core for building up a 55 larger diameter rod by winding on turns of resin-impregnated or resin-coated paper 31 and turns

of resin-impregnated textile material in the form of tape 32 from a reel 33.

Figure 9 shows a hank of cotton yarn 11 enclosed with a sheath or tube of woven material 35 and supported by a hook 12a while undergoing impregnation in a bath of an aqueous solution of a heat-hardenable phenol-formaldehyde condensation product.

Figure 10 shows the impregnated, sheathed enclosed yarn 35 after removal from the impregnating bath being passed through a die 14 for the removal of surplus liquid.

Figure 11 is similar to Figure 6 and shows the twisting and tensioning of the sheathed and impregnated yarn 35 by means of the weighted bar 23 which has been locked against untwisting by the insertion of posts 28, 29 in the sockets 26 and 27.

#### Example

2,500 ends of 60's counts cotton yarn 11, supported as at 12 are impregnated by dipping, in the hank form, into an aqueous solution of a bath 13 of heat-hardenable phenol-formaldehyde condensation product made by reacting phenol and aqueous formaldehyde in the presence of an alkaline condensing agent. The surplus liquid may be removed by passing the impregnated hank 11 through a die 14 (Figure 2) or through a pair of squeeze rolls 15, 16 in which the gap is so adjusted that the product when subsequently dried contains approximately 60 parts of resin and 40 parts of cotton. The impregnated hank is dried for 30 minutes at 110° C. as shown in Figure 4 and is then suspended from a support in an oven 21 (Figures 5 and 6) and at the same time subjected to a tension of 56 pounds by means of a weight 22 attached to the bottom of the hank and provided with ready means for rotating and locking against rotation (as bar 23). Immediately after the application of the load, the impregnated hank is twisted by rotating the weight 22 by means of bar 23 (Figure 6) in such a manner that the threads are twisted through 60° per inch of length. The twisted hank is locked by posts 28 and 29 and is heated under tension for 2 hours at 120° C. to harden the resinous binder. After removal of the resinous surface by any of the conventional machining methods (as diagrammatically shown in Figure 7), a finished rod of approximately 0.25 inch diameter is produced. A rod (partly shown at 30, Figure 7) made in the manner described above may, if desired, be utilised either in the cured or semi-cured form, as a core in the production of a larger diameter rod by winding on it a suitable number of turns of impregnated or coated paper and/or textile material as indicated in Figure 8 and hardening by one of the conventional methods.

#### We claim:

1. A process for the manufacture of rods with solid cores comprising bonded fibrous material, which process comprises treating, with a bonding agent, longitudinally-arranged fibrous elements, and applying tension and twist simultaneously to a bundle of the said treated fibrous elements while solidifying the bonding agent to form a rod having a solid core.

2. A process for the manufacture of rods with solid cores comprising bonded fibrous material, which process comprises treating, with a bonding agent, longitudinally-arranged fibrous elements, a bundle of the said fibrous elements being enclosed in a sheath or tube permeable to the bonding agent and applying tension and twist simultaneously to the sheathed and treated fibrous ele-

ments while solidifying the bonding agent to form a rod having a solid core.

3. A process for the manufacture of rods with solid cores comprising bonded fibrous material, which process comprises treating, with a heat-hardenable bonding agent, longitudinally-arranged fibrous elements applying tension and twist simultaneously to a bundle of the said treated fibrous elements, winding fibrous material treated with a heat-hardenable bonding agent around the said twisted bundle of fibrous elements and applying heat to effect hardening of the bonding agent while maintaining the wound fibrous material under tension and twist to form a rod having a solid core.

4. A process for the manufacture of rods with solid cores comprising bonded fibrous material, which process comprises treating, with a heat-hardenable bonding agent, longitudinally-arranged fibrous elements, applying tension and twist simultaneously to a bundle of the said treated fibrous elements, heating to harden the bonding agent while the fibrous material is subjected to tension and twist to form a rod having a solid core, winding fibrous material treated with a heat-hardenable bonding agent around the rod and applying heat to effect hardening of the bonding agent.

5. A process for the manufacture of rods with solid cores comprising bonded fibrous material, which process comprises treating, with a liquid heat-hardenable bonding agent, longitudinally-arranged fibrous elements, removing surplus liquid from the fibrous elements, drying the said fibrous elements and applying tension and twist simultaneously while heating to effect hardening of the bonding agent to form a rod having a solid core.

6. A process for the manufacture of rods with solid cores comprising bonded fibrous material, which process comprises treating, with a bonding agent, longitudinally-arranged fibrous elements, applying tension and twist simultaneously to a bundle of the said treated fibrous elements while solidifying the bonding agent to form a rod having a solid core, the said bonding agent being an inorganic bonding agent.

7. A process for the manufacture of rods with solid cores comprising bonded fibrous material, which process comprises treating, with a bonding agent, longitudinally-arranged fibrous elements, applying tension and twist simultaneously to a bundle of the said treated fibrous elements while solidifying the bonding agent to form a rod having a solid core, the said bonding agent being an organic bonding agent.

8. A process for the manufacture of rods with solid cores comprising bonded fibrous material, which process comprises treating, with a thermoplastic resinous bonding agent, longitudinally-arranged fibrous elements, applying tension and twist simultaneously to a bundle of the said treated fibrous elements while applying heat to bring about effective bonding of the fibrous elements, and solidifying the resin while maintaining the bundle under twist and tension to form a rod having a solid core.

9. A process for the manufacture of rods with solid cores in continuous lengths which rods comprise longitudinally-arranged fibrous elements bonded together, the process comprising moving an assembly of the said fibrous elements through a liquid containing heat-hardenable resin, removing surplus liquid from the assembly, drying the impregnated assembly under conditions that pre-

clude the hardening of the resin, subjecting the assembly to twist and tension simultaneously and while subjected to such twist and tension hardening the resin by heating to form a rod having a solid core.

10. A process for the manufacture of rods with solid cores which rods comprise longitudinally-arranged fibrous elements bonded together with heat-hardenable bonding agent which process comprises treating an assembly of the said fibrous elements with an aqueous liquid containing the bonding agent, removing surplus liquid from the fibrous elements, removing water from the assembly of elements by heating, subjecting the assembly to tension and twist and at the same time to heat so as to harden the bonding agent thereby forming a rod with a solid core, machining the rod, wrapping the machined rod with fibrous material impregnated with heat-hardenable resin and hardening the material by heating.

11. A solid-core rod comprising a bonded assembly of tensed and twisted longitudinally-arranged fibrous elements, said assembly being characterized by rigidity and machineability.

12. A solid-core rod assembly of tensed and twisted longitudinally-arranged fibrous elements impregnated and bonded with synthetic resin, said assembly being characterized by rigidity and machineability.

13. A solid-core rod assembly of tensed and twisted longitudinally-arranged fibrous elements impregnated and bonded with heat-hardened synthetic resin, said assembly being characterized by rigidity and machineability.

NORMAN WATSON KNEWSTUBB. 35  
CHARLES ALEXANDER ROBB.

## REFERENCES CITED

The following references are of record in the file of this patent:

## UNITED STATES PATENTS

| Number     | Name               | Date           |
|------------|--------------------|----------------|
| Re. 19,019 | Metcalf            | Dec. 12, 1933  |
| 171,185    | Splitdorf          | Dec. 14, 1875  |
| 812,837    | Feder              | Feb. 20, 1906  |
| 928,266    | Morris             | July 20, 1909  |
| 1,203,896  | Morris             | Nov. 7, 1916   |
| 1,205,376  | Morris             | Nov. 21, 1916  |
| 1,392,535  | Stevenson          | Oct. 4, 1921   |
| 1,411,786  | Hopkinson          | Apr. 4, 1922   |
| 1,567,574  | Clay               | Dec. 29, 1925  |
| 1,654,944  | Penfold et al.     | Jan. 3, 1928   |
| 1,923,168  | Simmons            | Aug. 22, 1933  |
| 2,055,776  | Saladino           | Sept. 29, 1936 |
| 2,104,730  | Bjorkman           | Jan. 11, 1938  |
| 2,158,771  | Beckwith           | May 16, 1939   |
| 2,210,432  | Roesch             | Aug. 6, 1940   |
| 2,220,958  | Jennings           | Nov. 12, 1940  |
| 2,243,917  | Owens              | June 3, 1941   |
| 2,245,824  | Roesch             | June 17, 1941  |
| 2,288,072  | Collins            | June 30, 1942  |
| 2,349,975  | Mackenzie          | May 30, 1944   |
| 2,363,871  | Keen et al.        | Nov. 28, 1944  |
| 2,364,134  | Dow et al.         | Dec. 5, 1944   |
| 2,379,881  | Chamberlain        | July 10, 1945  |
| 2,419,328  | Watson             | Apr. 22, 1947  |
| 2,427,507  | Powell, 3d, et al. | Sept. 16, 1947 |